

## UNITED STATES PATENT OFFICE

2,379,783

METHOD FOR THE PRODUCTION OF A  
HOLLOW TEXTILE MATERIAL

Orlow William Boies, Wethersfield, and Harold  
Oliver Taylor, Rocky Hill, Conn., assignors to  
The Hartford Rayon Corporation, Rocky Hill,  
Conn., a corporation of Delaware

No Drawing. Application July 8, 1941,  
Serial No. 401,520

9 Claims. (Cl. 106—122)

The invention relates to a method for the production of a hollow textile material. More particularly, it pertains to the preparation of a hollow filament adapted for the manufacture of textiles, and includes correlated improvements and discoveries whereby the qualities of such filaments are enhanced.

It is an object of the invention to provide a method for the production of a synthetic or artificial textile material.

A further object of the invention is the provision of a method for the production of a so-called hollow filament, i. e., a filament having a multiplicity of voids or gas filled vesicles, utilization being made of a solution of a coagulatable material containing a compound which reacts with another compound in a coagulating bath, with release of a gas which is retained within the body of the formed filament, imparting thereto the characteristics of a hollow filament.

An additional object of the invention is to provide a method for the manufacture of a hollow filament which may be readily, effectively and economically carried out on a commercial scale and to a desired extent.

A specific object of the invention is the provision of a procedure whereby a hollow filament may be produced from viscose.

Other objects of the invention will in part be obvious and will in part appear hereinafter.

The invention accordingly comprises the several steps and the relation of one or more of such steps with respect to each of the others thereof, which will be exemplified in the process hereinafter disclosed, and the scope of the invention will be indicated in the claims.

In the practice of the invention a textile material of the hollow type, more particularly a hollow filament, may be produced from a composition containing a coagulatable material, as cellulose xanthate, nitrate, acetate and the like, and a cuprammonium solution of cellulose in conjunction with a substance capable of reacting, as with an acid, in a coagulating bath, with evolution of a gas, and finally coagulating in a suitable medium or bath. More particularly, there may be prepared a solution containing a strong alkali, for example, sodium and potassium hydroxides, and a carbonate which may be soluble or insoluble in water, admixing cellulose xanthate therewith to form a coagulatable solution, and coagulating in an acid bath.

As a carbonate utilization may be made of the carbonates of sodium, potassium, ammonium, calcium, magnesium and the like, and when the

carbonate is insoluble in water it may be employed as a suspension therein. Moreover, the carbonate may be in the form of a normal or of a bi-carbonate, with preference attending the use of the normal carbonates, as sodium carbonate  $Na_2CO_3$ . As above stated, coagulation of such a composition leads to the formation of a material, as a filament, having a multiplicity of voids or gas filled pockets which give the product a hollow appearance. If desired, a delusterer, as an oxide of titanium, and a lubricant, as a mineral oil, may be incorporated with the alkali-carbonate solution prior to admixing the coagulatable material, as the xanthate, therewith. Somewhat more particularly as to details the procedure entails preparing an alkali cellulose through a shredding of a cellulose and treatment with a strong alkali, e. g., sodium hydroxide, followed by ripening. The alkali cellulose may then be converted into a xanthate by treatment with carbon disulfide, and this xanthate admixed with a solution containing sodium hydroxide and a carbonate. The admixture so produced may then be ripened with attending deaeration, and then coagulated, as by spinning in an acid bath.

As an illustrative embodiment of a manner in which the invention may be practiced, the following description is presented. Cellulose, as wood pulp in the form of sheets, is treated with a solution of sodium hydroxide having a concentration of about 17.6%, at a temperature of from about 16.5 to 17.5° C. This treatment may continue for a period of about one hour whereupon the excess caustic liquor is removed by pressing, and the alkali cellulose formed is shredded. Shredding of the alkali cellulose, which may require a period of about two hours, during which temperature may rise to from 24—29° C., reduces the alkali cellulose to crumbs, which are then aged at a temperature of 21—23° C. Aging of the alkali cellulose is followed by conversion into a xanthate, e. g., by treatment with carbon disulfide in a temperature range from 24—30° C., and for a period of about two hours. There is also prepared a solution of a strong alkali, preferably sodium hydroxide, in a concentration of 3.6%, and to this there is added a carbonate, as sodium carbonate.

By way of illustration, to each 845 liters of 3.6% sodium hydroxide there may be added 99 lbs. of sodium carbonate. The mass is agitated until solution has been effected. If desired, there may now be added to the sodium hydroxide-sodium carbonate solution a delusterer, as titanium dioxide, in an amount of about 3.25 lbs., and a lubricant, as a mineral oil, in an amount

of about 6 lbs. These amounts are introduced into a volume of about 845 liters of the solution. Following mixing for a period of about thirty minutes at a temperature of about 17° C. cellulose xanthate is added to form viscose, and the charge is mixed for a period upwards of eight hours, i. e., not less than eight hours. The viscose may now be filtered and a vacuum applied for about twelve to fourteen hours at 17° C.

Following aging for a total period of about twenty-four to twenty-eight hours the viscose may again be filtered, and is then spun by introducing into a suitable coagulating bath, as an acid bath containing sulfuric acid or sulfuric acid in conjunction with sodium sulfate. If desired, other acids, as hydrochloric and phosphoric, may be utilized in place of or in conjunction with sulfuric acid. The viscose solution is characterized by having a total alkalinity, expressed as sodium hydroxide of 8.95%; a cellulose content of 7.55%; a viscosity of 37.5 seconds by the falling sphere method; sodium carbonate 3.6%; titanium oxide 0.199%; and mineral oil 0.225%. Spinning of the viscose solution may be through a spinneret having orifices with diameters of about 0.008", and the denier when so spun is about 600. The spinning bath may have a titration value of 15.0 cc. normal sodium hydroxide, a specific gravity of 1.302, and concentrations of acid, sodium sulfate and zinc sulfate of 11, 25 and 0.64% respectively. The temperature of the spinning bath may be from 45 to 47° C., and following spinning the yarn obtained is processed in the usual manner, i. e., washed, dried, twisted, reeled, bleached, again dried, inspected and packed for the market.

The foregoing procedure leads to the production of a textile material, especially a filament of the so-called hollow tube type, inasmuch as the body of the material contains a multiplicity of voids or pockets produced by reaction in the acid bath, giving rise to a gas. It may be mentioned more particularly that the gas producing compound, as a carbonate, is incorporated with the sodium hydroxide or strong alkali solution prior to the introduction of the xanthate thereto. By so doing applicants obtain a hollow material possessing satisfactory qualities, not only from the standpoint of various processings during the fabrication of textile materials therefrom, but also in regard to the appearance and feel or hand of the product while in yarn or other form, and also when forming the whole or part of a finished textile.

Since certain changes may be made in carrying out the above process without departing from the scope of the invention, it is intended that all matter contained in the above description shall be interpreted as illustrative and not in a limiting sense.

It is also to be understood that the following claims are intended to cover all of the generic and specific features of the invention herein described, and all statements of the scope of the invention which, as a matter of language, might be said to fall therebetween.

Having described our invention, what we claim as new and desire to secure by Letters Patent, is:

1. A method for the preparation of a spinning solution for hollow textile material, which comprises preparing a solution containing an alkali metal hydroxide and a carbonate, and then ad-

mixing a coagulable material belonging to the group consisting of cellulose esters and a cuprammonium solution of cellulose therein.

2. A method for the preparation of a spinning solution for hollow textile material, which comprises preparing a solution of an alkali metal hydroxide, incorporating a carbonate of sodium therein, and then admixing a coagulable material belonging to the group consisting of cellulose esters and a cuprammonium solution of cellulose therewith.

3. A method for the preparation of a spinning solution for hollow textile material, which comprises preparing a solution of sodium hydroxide, incorporating a carbonate of sodium therein, and then admixing cellulose xanthate therewith to form a spinnable solution.

4. A method for the preparation of a spinning solution for hollow textile material, which comprises preparing an alkali cellulose, converting said alkali cellulose into a xanthate, preparing a solution containing an alkali metal hydroxide and a carbonate, and then admixing the xanthate therewith to form a spinnable solution.

5. A method for the preparation of a spinning solution for hollow textile material, which comprises preparing an alkali cellulose, converting said alkali cellulose into a xanthate, preparing a solution containing sodium hydroxide and a carbonate of sodium and then admixing the xanthate therewith to form a spinnable solution.

6. A method for the preparation of a spinning solution for hollow textile material, which comprises preparing an alkali cellulose, converting said alkali cellulose into a xanthate, preparing a solution containing an alkali metal hydroxide and a carbonate, adding thereto a delusterer and a lubricant, and then admixing the xanthate therewith to form a spinnable solution.

7. A method for the preparation of a spinning solution for hollow textile material, which comprises preparing an alkali cellulose, converting said alkali cellulose into a xanthate, preparing a solution containing an alkali metal hydroxide and a carbonate, adding thereto an oxide of titanium and a mineral oil, and then admixing the xanthate therewith to form a spinnable solution.

8. A method for the preparation of a spinning solution for hollow textile material, which comprises preparing an alkali cellulose, converting the alkali cellulose into xanthate by treatment with carbon disulfide, preparing a solution containing sodium hydroxide and sodium carbonate; then admixing the xanthate therewith, and ripening the admixture with attending de-aeration.

9. A method for the preparation of a spinning solution for hollowing filament, which comprises preparing an alkali cellulose, converting the alkali cellulose into xanthate by treatment with carbon disulfide at a temperature of about 24-30° C. for a period of about two hours, preparing a solution containing sodium hydroxide and sodium carbonate, then admixing the xanthate therewith for a period upwards of eight hours, and ripening the admixture with attending de-aeration at a temperature of about 17° C. for a period of about twenty-four to forty-eight hours.

ORLOW WILLIAM BOIES.  
HAROLD OLIVER TAYLOR.